

Feb. 24, 1925.

1,527,659

W. WILKIE

CAPSULE AND METHOD OF FORMING THE SAME

Filed Nov. 19, 1923

Fig. 1. Fig. 2. Fig. 3. Fig. 4. Fig. 5. Fig. 6.



Fig. 7.



Fig. 8.



Fig. 9.



Inventor

Warren Wilkie

By Whitemore Hubert Whitemore

Dechamph

Attorneys

Patented Feb. 24, 1925.

## UNITED STATES PATENT OFFICE.

WARREN WILKIE, OF DETROIT, MICHIGAN, ASSIGNOR TO PARKE, DAVIS & COMPANY,  
OF DETROIT, MICHIGAN, A CORPORATION OF MICHIGAN.

## CAPSULE AND METHOD OF FORMING THE SAME.

Application filed November 19, 1923. Serial No. 675,779.

*To all whom it may concern:*

Be it known that I, WARREN WILKIE, a citizen of the United States of America, residing at Detroit, in the county of Wayne 5 and State of Michigan, have invented certain new and useful Improvements in Capsules and Methods of Forming the Same, of which the following is a specification, reference being had therein to the accompanying drawings.

The invention relates to the manufacture of capsules or ampoules for containing a medicinal agent and it is the object of the invention to obtain a construction having 10 chemical and physical properties which peculiarly adapt it for such use. One specific use of my improvement is for holding a solution of silver nitrate, but it is obvious that the construction is equally applicable to 15 other uses.

In the present state of the art capsules or ampoules for holding solutions of silver nitrate have been formed of glass, beeswax and other materials. Where made of glass, 20 the end must be fractured before the content is available and there is always danger of particles of glass being carried by the solution. Where made of beeswax, the end may be punctured and the content ejected by 25 squeezing the capsule, but it has been found that there is a chemical reaction between the beeswax and the silver nitrate solution which destroys the purity of the latter. Other waxy substances, such as paraffin, are 30 free from chemical reaction, but have not the physical characteristics for making a collapsible container. Thus if the walls are of sufficient thickness for strength, they 35 will be too brittle to permit of flexing.

To avoid the objections to the various constructions as above described, I have devised a capsule or ampoule having flexible walls with a lining which is chemically inert to the content. For the specific purpose of holding silver nitrate solution, this 40 capsule or ampoule is preferably of a composite form, including a thin walled lining of a chemically inert substance, such as paraffin or ceresin, and a surrounding heavy 45 wall of a more flexible and tougher material such as beeswax.

With this construction the silver nitrate comes in contact with the inner wall only and for a limited period of time it will remain entirely pure. However, upon aging 50

it has been found that even in these capsules decomposition of the silver nitrate takes place with the formation of free nitric acid and experimentation has revealed that this is due to the permeation of the beeswax 60 through the paraffin. To avoid this condition it is preferable to interpose between the outer wall and inner lining a coating of material resistant to the action of the beeswax. I have discovered that a number of 65 materials may be employed for this purpose, such as shellac, sandarac, copal or other gum solution and collodion or other esters of cellulose, these materials effectively isolating the beeswax from the liquid within 70 the inner lining.

My preferred form of capsule, therefore, consists of an outer coating of beeswax to 75 secure the proper degree of toughness and flexibility so that it may be squeezed or pierced without crumbling; an inner coating of some neutral mineral wax such as paraffin or ceresin to avoid chemical security for the contents of the capsule; and a protective lining or coating between the two 80 that will isolate the two waxes and prevent beeswax from permeating either the mineral wax or any air bubbles or other fissures in the same. I have also devised a process of manufacturing and filling such capsules as 85 hereinafter more fully set forth.

In the drawings:

Figures 1 to 8 show in longitudinal section the various stages of manufacturing and filling the capsule or ampoule; 90

Figure 9 is a perspective view of the completed capsule.

My improved composite capsule or ampoule may be formed by dipping a tapering pin A (Figure 1) into a solution of 95 melted paraffin, ceresin or some other neutral mineral wax so as to form thereon a thin adhering coating B, preferably about  $\frac{1}{2}$  of an inch in thickness. The pin A is then dipped into a vessel containing a protective material such as shellac, sandarac, copal or other gum solution or collodion or other esters of cellulose, this operation forming a thin film C of protecting material 100 around the inner coating B. The pin A is then dipped once again, this time in melted beeswax, to form a surrounding coating D of greater thickness, preferably  $\frac{1}{16}$  of an inch but leaving at the upper end a projecting portion of the thin material forming 105

the inner lining B. The composite structure may then be stripped from the pin and the capsule filled with the desired content E, such as silver nitrate, after which the projecting portion F of the inner lining is squeezed together as indicated at G to close the opening. This is sealed by fusing the ends of the adjacent walls together, after which the upper end of the capsule is again 10 dipped into the shellac or other protective material and then into beeswax to complete the outer coating of the capsule.

The capsule or ampoule formed as described can be kept indefinitely without any injury to the content, inasmuch as the lining or paraffin or ceresin has no deleterious effect upon the silver nitrate while the protective coating of shellac or other material prevents any penetration of the 20 beeswax through the inner lining. The outer beeswax coating imparts the toughness and flexibility to the capsule so that whenever it is desired to eject the content the end may be perforated, after which the 25 walls may be collapsed to force out the solution.

What I claim as my invention is:—

1. A composite capsule or ampoule comprising a thin inner wall of a material chemically inert to the content, said inner wall being closed and sealed at its filling end and a surrounding coating of a tougher and flexible material.

2. A capsule or ampoule comprising an inner wall of a material chemically inert to the content and of sufficient thinness to be flexible, said inner wall being hermetically sealed at its filling end and a surrounding coating forming a thicker supporting wall 40 of a material having greater flexibility and toughness.

3. A capsule or ampoule comprising an inner wall of a material chemically inert to the content and of sufficient thinness to be flexible, being collapsed and sealed at its filling end, and a surrounding coating forming a wall of greater thickness and of a material having greater flexibility and toughness.

4. A capsule or ampoule comprising an inner wall of a material such as paraffin of sufficient thinness to be flexible and closed and sealed at its filling end, and a surrounding non-metallic coating forming an outer wall of greater thickness of a material of a more 55 flexible and tougher nature.

5. A silver nitrate capsule or ampoule comprising an inner wall of a material such as paraffin of sufficient thinness to be flexible and sealed at its filling end, and a surrounding coating of beeswax forming a thicker reinforcing wall.

6. A composite capsule or ampoule comprising a thin inner wall of a material chemically inert to the content, a surrounding coating of a tougher and flexible ma-

terial, and an intermediate lining of a material preventing the permeation of the latter into the former.

7. A capsule or ampoule comprising an inner wall of a material chemically inert to the content and of sufficient thinness to be flexible, being collapsed and sealed at its filling end, a surrounding coating forming a wall of greater thickness and of a material having greater flexibility and toughness, and an intermediate lining of a material for preventing the permeation of the outer material into the inner material to such an extent as to injuriously affect the content of the capsule.

8. A capsule or ampoule comprising a flexible inner wall of a material chemically inert to the content, such as paraffin, a surrounding coating of beeswax forming a thicker reinforcing wall, and an intermediate lining between said outer and inner walls for preventing the penetration of the beeswax into the inner material.

9. The method of forming capsules or ampoules comprising the dipping of a mold into a molten material to form a thin walled coating, and redipping the coated mold into a different molten material to form a thicker reinforcing coating.

10. The method of forming capsules or ampoules comprising the dipping of a mold into a molten material to form a thin walled coating, redipping the coated mold into another molten material to form a surrounding reinforcing wall, leaving a projecting portion of the thin wall, filling the container, collapsing the projecting thin walls and sealing the same, and coating the projecting thin walled portion to complete the surrounding reinforcing wall.

11. The method of forming capsules or ampoules comprising the dipping of a mold in a molten material such as paraffin to form a thin coating thereon, redipping the coated mold into a molten material such as beeswax to form a thicker reinforcing wall with a projecting portion of the thin wall, stripping the composite structure from the mold, filling, collapsing the projecting thin walled portion and sealing the same, and coating said projecting portion with a beeswax to complete the reinforcing wall.

12. The method of forming capsules or ampoules comprising the dipping of a mold into a fluid material to form a thin wall coating, redipping the coated mold into a different fluid material to form a protective film thereon, and again dipping the mold into a third fluid material to form a thicker reinforcing coating.

13. The method of forming capsules or ampoules comprising the dipping of a mold in a fluid material, such as paraffin, to form a thin coating thereon, redipping the coated mold into a fluid for protecting said coating,

again dipping the coated mold into a third material, such as molten beeswax, to form a thicker reinforcing wall with a projecting portion on the inner wall, stripping the 5 composite structure from the mold, filling collapsing the projecting inner portion and sealing the same, redipping the sealed por-

tion of said capsule into the second mentioned material and finally coating said projecting portion with beeswax to complete the 10 reinforcing wall.

In testimony whereof I affix my signature.

WARREN WILKIE.